# EUROPEAN PATENT SPECIFICATION

(11) **EP 4 320 298 B1**
(45) Date of publication and mention of the grant of the patent: **04.03.2026**
(21) Application number: 22783735.8
(22) Date of filing: 07.04.2022
(51) Int. Cl.: D03D 15/00, A41D 31/02, A41D 31/10, D03D 15/50, D03D 15/208, D03D 15/283, D03D 15/527, D03D 23/00, D06M 17/00

(54) **NO SWEAT MARKS FABRIC WITH MOISTURE MANAGEMENT FUNCTION**
SCHWEISSFREIES GEWEBE MIT FEUCHTIGKEITSMANAGEMENTFUNKTION
TISSU DÉPOURVU DE MARQUES DE TRANSPIRATION AYANT UNE FONCTION DE GESTION DE L'HUMIDITÉ

(30) Priority: 09.04.2021 US 202163173093 P
(43) Date of publication of application: 14.02.2024
(73) Proprietor: Lululemon Athletica Canada Inc., Vancouver, British Columbia V6Z 2K2 (CA)
(72) Inventor: DANDAPURE, Yogendra V, Vancouver, British Columbia V6Z 2K2 (CA); LOGAN, Peter Crombie, Vancouver, British Columbia V6Z 2K2 (CA); MANNA, Rovin, Vancouver, British Columbia V6Z 2K2 (CA)
(74) Representative: Regimbeau
(86) International application number: PCT/CA2022/050529
(87) International publication number: WO 2022/213199

(56) References cited:
- EP-A1- 0 431 984
- JP-A- 2005 146 485
- US-A- 5 312 667
- US-A1- 2003 181 118
- US-A1- 2005 016 614
- US-A1- 2007 093 162
- US-A1- 2008 096 001
- US-A1- 2019 234 013
- US-B2- 7 682 994
- MONTALVO J G ET AL: "Review of Standard Test Methods for Moisture in Lint Cotton", THE JOURNAL OF COTTON SCIENCE, 1 January 2008 (2008-01-01), pages 33 - 47, XP093217917, Retrieved from the Internet <URL:https://www.cotton.org/journal/2008-12/1/upload/JCS12-33.pdf> [retrieved on 20241024]

## Description

### CROSS-REFERENCE TO RELATED APPLICATIONS

The present application is claiming priority from U.S. Provisional Application No. 63/173,093 filed April 9, 2021.

### TECHNICAL FIELD

It is provided a fabric with moisture management function that reduces occurrence of moisture (liquid) spots, such as sweat spots, water spots or blood spots on its face surface.

### BACKGROUND

Fabrics used in apparel designed for athletic activities are conceived with the objective of maximizing the body performance by notably controlling the body temperature and keeping the moisture away from the individual. The challenge is to manufacture such apparel which generally exhibit characteristics that enhance the performance without compromising the appearance and/or comfort of an individual. The moisture from the associated sweat generated as a result of physical exertion causes undesirable liquid spot on the face surface of the apparel. Having a fabric that reduces occurrence of moisture spots is convenient for wearers that can work out in a athletic gear and walk to get groceries or coffee without worrying about sweat marks. During hot humid days, people commuting desire to be provided with fabrics that would not show sweat marks on their clothing as well. Document US 2005/0016614 A1 discloses a moisture management double face woven fabric. Document US 2008/0096001 A1 discloses a breathable fabric. Document US 2007/0093162 A1 discloses a fabric and a method of making the fabric. Document EP 0 431 984 A1 discloses a double-faced elastic knitwear.

It is thus highly desired to be provided with improved fabrics that reduce occurrence of moisture spots on its face surface.

### SUMMARY

The invention is set out in the appended set of claims. In one aspect a knitted fabric with moisture management function is provided. The fabric comprises a face fabric layer with a durable water repellency (DWR) additives forming a fabric outer surface that is mostly hydrophobic, a back fabric layer comprising a second yarn that is hydrophilic forming a moisture regain core to absorb the moisture and spread it across on an inside surface of the back fabric layer, and a connecting yarn binding together the face fabric layer and the back fabric layer.

In an embodiment, the first yarn is spun using the DWR additives inside the yarn.

In another embodiment, the first yarn has the DWR additives finish.

In a supplemental embodiment, the fabric is a weft or warp knitted fabric.

In one aspect, the moisture regain of the back fabric layer is in the range of 4% - 18%.

In another aspect, the first yarn is a synthetic polymer selected from a group of a nylon, a polyester, a polypropylene, an acrylic or any blend or combination thereof.

In another embodiment, the first yarn is nylon 6.6 with denier range of 2 Tex to 11 Tex (20 D - 100 D) and number of filaments from 10 to 186.

According to the invention, the face fabric layer further comprises a third yarn knitted together with the first yarn such that the third yarn is on the inside and the first yarn is on the outside of the face fabric layer.

According to the invention, the second yarn comprises a natural or a regenerated cellulosic fiber selected from a group consisting of a cotton, silk, wool, modal, micro-modal, viscose rayon, lyocell, cupro, artificial silk, regenerated cellulosic fibers, regenerated protein fibers and any combination thereof.

According to the invention, the third yarn is an elastane.

According to the invention, the elastane has a yarn size in the range of 1 Tex to 8 Tex (10 D to 70 D).

In a supplemental embodiment, the face fabric layer is a composite blend of a synthetic polymer with the DWR additives plaited with an elastane.

According to the invention, the back fabric layer further comprises a fourth yarn joined together with the second yarn such that the fourth yarn is on the inside and the second yarn is on the outside of the back fabric layer.

According to the invention, the second yarn is a hydrophilic synthetic polymer selected from a group consisting of a nylon, a modified polyester, a modified polypropylene, a modified acrylic and a combination thereof.

According to the invention, the fourth yarn is an elastane.

According to the invention, the elastane has a yarn size in the range of 1 Tex to 8 Tex (10 D to 70 D).

In another embodiment, the second fabric layer is a composite blend of a natural fiber or a regenerated cellulosic fiber plaited with an elastane.

In a further embodiment, the back fabric layer is peached or brushed to increase its surface area.

In another aspect, the connecting yarn is at least a single strand.

In a further embodiment, the connecting yarn is a synthetic polymer.

According to the invention, the connecting yarn is an elastane.

In another aspect, an outer surface of the face fabric layer is finished with a durable water repellency (DWR) coating.

In another aspect, an outer surface of the back fabric layer comprises a wicking finish.

In one aspect, the fabric is knitted from a double jersey plaited construction.

In one aspect the fabric is a plaited single jersey fabric.

In one aspect the fabric is a plaited warp knitted fabric.

In one aspect not according to the invention, the fabric is a double weave woven fabric.

In another embodiment, the fabric is a piqué fabric or a tricot fabric.

In one aspect, an article of apparel comprising the fabric as defined herein is provided.

### BRIEF DESCRIPTION OF THE DRAWINGS

Reference will now be made to the accompanying drawings.
Fig. 1 illustrates a schematic representation of a double jersey plaited construction fabric as encompassed herein in accordance to an embodiment.
Fig. 2 illustrates a schematic representation of a no-sweat piqué fabric showing the four courses or repeat that makes the piqué.
Fig. 3 illustrates a double weave fabric not according to the invention.
Fig. 4 illustrates a tricot fabric construction encompassed herein in accordance to an embodiment.

### DETAILED DESCRIPTION

In accordance with the present disclosure, it is provided a knitted fabric with moisture management function comprising a face fabric layer with a first yarn that has durable water repellency (DWR) additives or a DWR finish forming an outer surface that is hydrophobic or mostly hydrophobic, a back fabric layer comprising a second yarn that is highly hydrophilic forming a moisture regain core to absorb the moisture and spread it across on an inside surface of the back fabric layer, and a connecting yarn binding together the face fabric layer and the back fabric layer. The moisture that is absorbed and spread across the inside surface between the back fabric layer and the face fabric layer evaporates over time through the face fabric layer. The outer (face) layer of the fabric is hydrophobic due to the added DWR additives or DWR finish to the first yarn while the inner (back) layer of the fabric is hydrophilic that absorbs and spreads the moisture across the inner side of the back layer so that it dries faster making the outer surface of the face fabric layer dry thus avoiding or reducing the occurrence of liquid spots on the face layer outer surface.

As seen in Fig. 1, the fabric 10 comprises a back (inner) layer 12 which is the layer next to the skin of a wearer and a face (outer) layer 14 which correspond to the layer of the fabric 10 facing the exterior and away from the skin of the wearer. As illustrated in Fig. 1, in an embodiment, a connecting yarn 16 binds together the back fabric layer 12 and the face fabric layer 14 connecting the fabric 10 together. The moisture from a wearer skin is pushed through the back fabric layer 12 and it will spread on the backside of the fabric 10, essentially from side A (the skin of the wearer face) towards B (the exterior face and away from the skin of the wearer). The absorbed moisture spread therein evaporates out over the time without making sweat marks showing on the face 14 of the fabric 10.

The face fabric layer 14 comprises a first yarn 23 that comprises the durable water repellency (DWR) additives or DWR finish therein thus forming a fabric outer surface that is hydrophobic thus avoiding or reducing the occurrence of a sweat mark on the outer surface of the fabric 10 during sweaty activities. For example, the first yarn 23 can be spun using a DWR additives inside the yarn 23 or the yarn 23 can have a DWR finish. The back fabric layer 12 comprises a second yarn 18 that is hydrophilic forming a moisture regain core that absorbs the moisture from the skin and spreads it across on an inside surface of the back fabric layer therefore making it dry faster while keeping the outer surface of the face layer 14 without sweat mark visible on the outside of the fabric 10.

In the illustrated embodiment of Fig. 1, the face fabric layer 14 further comprises a third yarn 24 knitted or woven together with the first yarn 23 such that the third yarn 24 is on the inside while the first yarn 23 is on the outside of the face layer 14. In some implementations, the first yarn 23 can be a synthetic polymer, such as for example but not limited to, a nylon, a polyester, a polypropylene, an acrylic or any bland combination thereof. In one embodiment, the first yarn 23 can be a 1.7 Tex to 11 Tex (15 to 100 denier(D))/ 10 to 184 filaments (F) 6.6 nylon with DWR additives. The third yarn 24 is an elastane, having a yarn size in the range Tex to 8 Tex (10D to 70D) . The face fabric layer 14 can be a composite blend of a synthetic polymer with DWR additives plaited with an elastane or with DWR finish. In various embodiments, the outer surface of the face layer 14 comprises DWR finish.

The back fabric layer 12 comprises a second yarn 18 that is hydrophilic forming a high moisture regain thus forming a hydrophilic moisture regain core of the fabric 10. For example, the moisture regain of the second yarn 18 can be in a range of 4% - 18%. The second yarn 18 can be any suitable natural fiber or a regenerated cellulosic fiber. For example, the second yarn 18 is selected from a group consisting of a cotton, silk, wool, modal, micro-modal, viscose rayon, lyocell, cupro, artificial silk and any combination thereof. In some implementations, not according to the invention, the second yarn 18 can be hydrophilic synthetic polymer, such as for example, the second yarn 18 can be selected from a group consisting of a nylon, a polyester, a polypropylene, an acrylic and a combination thereof. The back fabric layer 12 further comprises a fourth yarn 20 knitted together with the second yarn 18 such that the fourth yarn 20 is on the inside and the second yarn 18 is on the outside of the back fabric layer 12. The fourth yarn 20 is an elastane. For example, the fourth yarn 20 can be 3 Tex or 4 Tex (30D or 40D) spandex. In one embodiment, the back fabric layer 12 can be a composite blend of a natural fiber, hydrophilic synthetic polymer or a regenerated cellulosic fiber plaited with an elastane. In a manner not according to the invention, the face DWR and back side hydrophilic yarns can be on their own without any plaiting with spandex. In another embodiment, the back fabric layer 12 can be a composite blend of a fully hydrophilic synthetic polymer, such as nylon, plaited with an elastane. One means to increase the hydrophilic nature of the back layer 12 is to increase its surface area. Accordingly, it is encompassed that an outer side (facing skin) of the back fabric layer 12 can be peached or brushed to increase its surface area.

The connecting yarn 16 is binding together the face fabric layer 14 and the back fabric layer 12 and is a single strand elastane. For example, the connecting yarn 16 can be 1 Tex to 8 Tex (10D to 70D) spandex. In some implementations, not according to the invention, the connecting yarn 16 can be a synthetic polymer such as for example a nylon, a polyester, a polypropylene, an acrylic, a polyacrylic or a combination thereof. Alternatively, the connecting yarn 16 can be a natural fiber such as for example a cotton, silk, wool, modal, micro-modal, rayon, lyocell, viscose or a combination thereof. The connecting yarn is preferably a zig-zag structure between the back fabric layer 12 and the face fabric layer 14. The connecting yarn 16 is single strand. Each strand of the plurality of strands of the connecting yarn 16 can have independent zig-zag structure. The connecting yarn 16 can also be a yarn with DWR ingredient.

In one implementation, the outer surface of the face fabric layer 14 can be finished with a durable water repellency (DWR) coating to further reduce the occurrence of water or sweat spots on the outer surface of the fabric 10. For example, the DWR coating can be printed on the outer surface of the face fabric layer 14 once the face layer is finished. For example, the DWR coating can be printed, such as for example screen printed, inkjet printed, or laminated, or spray coated. In one implementation, the DWR coating can have a pre-determined pattern to provide moisture channelling out of the face layer 14 for faster drying. In one embodiment, the outer surface of the back fabric layer 12 can have a wicking finish, such as for example by adding a chemical finish containing a hydrophilic molecule that attaches to the outer surface of the back fabric layer 12.

In another example, not according to the invention, as depicted in Fig. 3, a double weave fabric is encompassed wherein a first yarn 23 is also connecting the face layer 14 with the back fabric layer 12. In this embodiment, the face layer 14 comprises yarns 23 finished with DWR. Thus, the double weave fabric comprises a backside of the fabric being hydrophilic and the face side with DWR yarn.

As described herein, in some embodiments, the described fabric 10 is made with a knitting construction which can be a weft knitted or warp knitted structure. For example, the fabric can be a double jersey plaited construction for example (as shown in Fig. 1) or Tricot warp knit structure (as shown in Fig. 4).

In an alternate example, not according to the invention, it is disclosed a fabric 100 wherein the back layer comprises an hydrophilic yarn 54 (Fig. 2). The hydrophilic yarn 54 in the illustrated embodiment is made of a natural fiber or a regenerated cellulosic fiber, preferably modal or a hydrophilic synthetic polymer. The connecting yarn 50 is a composite blend of a synthetic polymer with DWR additives plaited with an DWR finish. The face fabric layer comprises a yarn 52 and a face fabric or first yarn 56 knitted or woven together with the connecting yarn 50 such that the yarn 52 is on the inside while the first yarn 56 is on the outside of the face layer. The fabric 100 is knitted or "piqué". As encompassed herein, it is understood that piqué is a traditional woven style with a waffle-knit structure. The resulting double weave structure can be seen from the face fabric layer yarns having twice as many threads as the back layer yarns, thus creating raised and recessed areas in the material. This allows different patterns to be woven. In the illustrated implementation, the piqué construction is a repeat of four courses however there can be various iterations of this structure without departing from the scope of the invention. The first yarn 56 is a composite blend of a synthetic polymer with DWR additives plaited with an DWR finish. The yarn 52 is an elastane, such as for example 0.6 Tex (5D) spandex. A seen in Fig. 2, four courses or repeat are represented that makes it a piqué fabric 100.

As encompassed herein, the knitted fabric described herein with moisture management function and no sweat marks showing on its face can be used in any type of articles of apparel including shirts, headwear, coats, jackets, pants, underwear, gloves, socks, and footwear.

As demonstrated herein, the fabric properties were tested and the Moisture Management Test (MMT) results confirmed that the salt solution used during the testing didn't penetrate the fabric during the test. The fabric although blocks water, is air permeable, which is a preferable attribute when thermal comfort is concerned.

Based on the results, it is clear that fabric provided herein shows unique engineered moisture blocking property.

### EXAMPLE I

### Fabric tested properties

The liquid moisture management properties of textile fabric as depicted in Figures was tested using a Moisture Management Tester (MMT). The fabric was put between two layers of sensors (top and bottom layer of sensor) with the fabric face side facing downward. A salt solution of 0.2 ml was applied to the fabric back side (skin contact side of the fabric). Thus, "Top" is skin contact side/back side of fabric; "Bottom" is outer side/face side of fabric. The Table 1 below provides the results.

**Table 1:**

| Liquid moisture management indices | Average | Standard deviation | Grade* |
|---|---|---|---|
| Top wetting time, WTT (second) | 2.93 | 1.02 | 5 |
| Bottom wetting time, WTB (second) | 120 | 0 | 1 |
| Top absorption rate, ART (%/second) | 55.8 | 6.2 | 4 |
| Bottom absorption rate, ARB (%/second) | 0 | 0 | 1 |
| Top max wetting radius, MWRT (mm) | 25.0 | 0 | 5 |
| Bottom max wetting radius, MWRB (mm) | 0 | 0 | 1 |
| Top spreading speed, SST (mm/second) | 4.62 | 1.06 | 5 |
| Bottom spreading speed, SSB (mm/second) | 0 | 0 | 1 |
| One way transport capability, R (%) | -1100 | 50 | 1 |
| Overall moisture management capacity, OMMC | 0 | 0 | 1 |

| | | | |
|---|---|---|---|
| * Grade represents a textile grading from 1 to 5, 5 being the best that meets the desired function and 1 being the worst - does not conform to the desired outcome of a material. | | | |

The liquid absorption property of the fabric was tested wherein the back side (skin contact side) was in contact with the applied test liquid (distilled water). The liquid absorption rate by horizontal wicking (at 20-80% absorbent capacity) in gram per second was of 0.011.

As for the drying rate of the textile at its absorbent capacity, an air flow method was used. The test conditions were: air temperature - 21+1°C; relative humidity - 65+2%; air flow direction - vertical air flow from fabric back side to fabric face side; air speed before mounting the fabric - 2.5 + 0.5 m/s; and air speed after mounting the fabric - 0.10 m/s. What was observed is that water was unable to pass through the fabric.

A quick dry method was further used as this test method determines the drying rate of a fabric based on the evaporation rate that occurs at the approximate water absorbent capacity. Test specimen is mounted on a hoop. There is vertical air flow passing through the fabric (air flow perpendicular to the fabric surface).The higher the drying rate of the fabric, the better the drying performance it has. The test conditions were: air temperature - 21+1°C; relative humidity - 65+2%; temperature of hot plate - 37+1°C with fabric back side (skin contact side) in contact with hot plate; and air speed - 1.5±0.5 m/s (horizontal air flow over the surface of the fabric). The drying rate measured was of 1.66 mL/h.

In order to measure the fabric air permeability, a method was used to measure the drying rate of the fabric, exposed to a prescribed volume of water, while in contact with a heated plate set at 37 °C, the simulated skin surface temperature. There is horizontal air flow over the surface of fabric. The higher the drying rate of the fabric, the better the drying performance it has. At a test pressure of 125Pa over a 38 cm² test area, the following measurement were taken.

**Table 2:**

| | Unit | Value |
|---|---|---|
| Air Permeability Average | cfm | 34.8 |
| Air Permeability Maximum | cfm | 36.2 |
| Air Permeability Minimum | xfm | 33.8 |
| CV | % | 2.2 |

The total heat loss in a standard environment of fabric provided herein was tested at the following atmospheric conditions: an air temperature: 25.0+0.1°C; a relative humidity of 65+4% R.H.; for least 12 hours (specimen ≤ 5 mm thick) / At least 24 hours (specimen > 5 mm thick).

The actual test conditions were: air temperature - 25.0+0.1°C; relative humidity - 65+3% R.H.; air speed - 1.0±0.1 m/s (horizontal air flow over the surface of the fabric); temperature of hotplate - 35.0+0.1°C; and orientation of test specimen - specimens lied flat across the measurement unit with the side normally facing the human body towards the measuring unit. Fabric back side (skin contact side) is in contact with hotplate. Below are the values measured:

| | |
|---|---|
| Mean intrinsic thermal resistance of sample alone, Rcf (K×ₘ²/W): | 0.015 |
| Mean apparent intrinsic evaporative resistance of sample, *R*_{ef}^{A} (kPa×m²/W): | 0.002 |
| Total heat loss, *Q*ₜ (W/m²): | 796 |

While the disclosure has been described in connection with specific embodiments thereof, it will be understood that it is capable of further modifications and this application is intended to cover any variations, uses, or adaptations falling within the scope of the claims as come within known or customary practice within the art and as may be applied to the essential features hereinbefore set forth.

## Claims

1. A knit fabric (10) with moisture management function comprising:
a face fabric layer (14) comprising a first yarn (23), the first yam (23) having durable water repellency (DWR) additives or a DWR finish, wherein the first yarn (23) comprises a synthetic polymer, the first yarn (23) forming a face fabric layer outer surface that is mainly hydrophobic;
a back fabric layer (12) comprising a second hydrophilic yam (18) forming a moisture regain core to absorb a moisture and spread it across on an inner surface of the back fabric layer (12), whereby the second hydrophilic yarn (18) comprises natural fibers or regenerated cellulosic fibers;
wherein the face fabric layer (14) further comprises a third yarn (24) knitted together with the first yarn (23) such that the third yarn (24) is on an inner surface of the face fabric layer (14) and the first yam (23) is on the outer surface of the face fabric layer (14),
wherein the third yam (24) is an elastane and has a yarn size in a range of 1 Tex to 8 Tex (10 D to 70 D);
wherein the back fabric layer (12) further comprises a fourth yam (20) knitted together with the second yarn (18) such that the fourth yarn (20) is on an inner surface of the back fabric layer (12) and the second yarn (18) is on an outer surface of the back fabric layer (12), wherein the fourth yarn (20) is an elastane and has a yam size in a range of 1 Tex to 8 Tex (10 D to 70 D); and
a connecting yarn (16) binding together the face fabric layer (14) and the back fabric layer (12) in the knit fabric (10) such that the inner surface of the face fabric layer (14) faces the inner surface of the back fabric layer (12), wherein the connecting yarn (16) is a single strand elastane.

2. The knit fabric (10) of claim 1, wherein the first yarn (23) is spun using the DWR additives inside the yarn.

3. The knit fabric (10) of claim 1, wherein the outer surface of the face fabric layer (14) is finished with a DWR coating.

4. The knit fabric (10) of claim 1, wherein the synthetic polymer is selected from a group consisting of a nylon, a polyester, a polypropylene, an acrylic and any blend or combination thereof.

5. The knit fabric (10) of claim 4, wherein the synthetic polymer of the first yarn (23) is nylon 6.6, and the first yarn (23) has a yarn size in a range of 2 Tex to 11 Tex (20 D - 100 D) and number of filaments from 10 to 186.

6. The knit fabric (10) of any one of claims 1-4, wherein the outer surface of the face fabric layer (14) is peached or brushed.

7. The knit fabric (10) of any one of claims 1-6, wherein the fourth yarn (20) is a 3 Tex or 4 Tex (30D or 40D) elastane.

8. The knit fabric (10) of any one of claims 1-7, wherein the natural fibers or regenerated cellulosic fibers of the second yarn (18) are selected from a group consisting of a cotton, silk, wool, modal, micro-modal, viscose rayon, lyocell, cupro, artificial silk, regenerated cellulosic fibers, regenerated protein fibers, and any combination thereof.

9. The knit fabric (10) of any one of claims 1-8, wherein the connecting yarn (16) has a yarn size in the range of 1 Tex to 8 Tex (10 D to 70 D).

10. The knit fabric (10) of claim 9, wherein the connecting yarn (16) forms a zig-zag structure between the back fabric layer (12) and the face fabric layer (14).

11. The knit fabric (10) of any one of claims 1-10, wherein the fabric is a weft or warp knitted fabric.

12. The knit fabric (10) of claim 11, wherein the weft or warp knitted fabric has a plaited single jersey construction or a plaited double jersey construction.

13. The knit fabric (10) of any one of claims 1-12, wherein the outer surface of the back fabric layer (12) comprises a wicking finish.

14. The knit fabric (10) of any one of claims 1-11 or claim 13, wherein the fabric is a piqué fabric or a tricot fabric.

15. An article of apparel comprising the fabric (10) of any one of claims 1-14.

## Patentansprüche

1. Maschenware (10) mit Feuchtigkeitsmanagementfunktion, umfassend:
eine Obergewebeschicht (14), die ein erstes Garn (23) umfasst, wobei das erste Garn (23) Zusatzstoffe für dauerhafte Wasserabweisung (durable water repellency - DWR) oder eine DWR-Ausrüstung aufweist, wobei das erste Garn (23) ein synthetisches Polymer umfasst und das erste Garn (23) eine Obergewebeschicht-Außenoberfläche bildet, die hauptsächlich wasserabweisend ist;
eine Untergewebeschicht (12), die ein zweites, wasseranziehendes Garn (18) umfasst, das einen Feuchtigkeitsaufnahmekern bildet, um eine Feuchtigkeit zu absorbieren und sie über eine Innenoberfläche der Untergewebeschicht (12) zu verteilen, wobei das zweite, wasseranziehende Garn (18) Naturfasern oder regenerierte Zellulosefasern umfasst;
wobei die Obergewebeschicht (14) ferner ein drittes Garn (24) umfasst, das zusammen mit dem ersten Garn (23) gewirkt ist, derart dass das dritte Garn (24) sich auf einer Innenoberfläche der Obergewebeschicht (14) befindet und das erste Garn (23) sich auf der Außenoberfläche der Obergewebeschicht (14) befindet, wobei das dritte Garn (24) ein Elastan ist und eine Garngröße in einem Bereich von 1 Tex bis 8 Tex (10 D bis 70 D) aufweist;
wobei die Untergewebeschicht (12) ferner ein viertes Garn (20) umfasst, das zusammen mit dem zweiten Garn (18) gewirkt ist, derart dass das vierte Garn (20) sich auf einer Innenoberfläche der Untergewebeschicht (12) befindet und das zweite Garn (18) sich auf einer Außenoberfläche der Untergewebeschicht (12) befindet, wobei das vierte Garn (20) ein Elastan ist und eine Garngröße in einem Bereich von 1 Tex bis 8 Tex (10 D bis 70 D) aufweist; und
ein Verbindungsgarn (16), welches die Obergewebeschicht (14) und die Untergewebeschicht (12) in der Maschenware (10) derart aneinander bindet, dass die Innenoberfläche der Obergewebeschicht (14) der Innenoberfläche der Untergewebeschicht (12) zugewandt ist, wobei das Verbindungsgarn (16) ein Einzelfaden-Elastan ist.

2. Maschenware (10) nach Anspruch 1, wobei das erste Garn (23) unter Verwendung der DWR-Zusatzstoffe innerhalb des Garns gesponnen ist.

3. Maschenware (10) nach Anspruch 1, wobei die Außenoberfläche der Obergewebeschicht (14) mit einer DWR-Beschichtung ausgerüstet ist.

4. Maschenware (10) nach Anspruch 1, wobei das synthetische Polymer aus einer Gruppe ausgewählt ist, die besteht aus einem Nylon, einem Polyester, einem Polypropylen, einem Acryl und einer beliebigen Mischung oder Kombination davon.

5. Maschenware (10) nach Anspruch 4, wobei das synthetische Polymer des ersten Garns (23) Nylon 6.6 ist und das erste Garn (23) eine Garngröße in einem Bereich von 2 Tex bis 11 Tex (20 D bis 100 D) und eine Anzahl von Filamenten von 10 bis 186 aufweist.

6. Maschenware (10) nach einem der Ansprüche 1 bis 4, wobei die Außenoberfläche der Obergewebeschicht (14) leicht angeraut oder angeraut ist.

7. Maschenware (10) nach einem der Ansprüche 1 bis 6, wobei das vierte Garn (20) ein 3 Tex oder 4 Tex (30 D oder 40 D) Elastan ist.

8. Maschenware (10) nach einem der Ansprüche 1 bis 7, wobei die Naturfasern oder regenerierten Zellulosefasern des zweiten Garns (18) ausgewählt sind aus einer Gruppe, die besteht aus einem/einer Baumwolle, Seide, Wolle, Modal, Micro-Modal, Viskose Rayon, Lyocell, Cupro, Kunstseide, regenerierten Zellulosefasern, regenerierten Proteinfasern und einer beliebigen Kombination davon.

9. Maschenware (10) nach einem der Ansprüche 1 bis 8, wobei das Verbindungsgarn (16) eine Garngröße im Bereich von 1 Tex bis 8 Tex (10 D bis 70 D) aufweist.

10. Maschenware (10) nach Anspruch 9, wobei das Verbindungsgarn (16) eine Zickzackstruktur zwischen der Untergewebeschicht (12) und der Obergewebeschicht (14) bildet.

11. Maschenware (10) nach einem der Ansprüche 1 bis 10, wobei das Gewebe ein Schuss- oder Kettengewirk ist.

12. Maschenware (10) nach Anspruch 11, wobei das Schuss- oder Kettengewirk eine plattierte Single-Jersey-Konstruktion oder eine plattierte Double-Jersey-Konstruktion aufweist.

13. Maschenware (10) nach einem der Ansprüche 1 bis 12, wobei die Außenoberfläche der Untergewebeschicht (12) eine Ausrüstung mit Dochtwirkung umfasst.

14. Maschenware (10) nach einem der Ansprüche 1 bis 11 oder Anspruch 13, wobei das Gewebe ein Piqué-Gewebe oder ein Trikot-Gewebe ist.

15. Kleidungsstück, welches die Maschenware (10) nach einem der Ansprüche 1 bis 14 umfasst.

## Revendications

1. Tissu tricoté (10) avec fonction de gestion de l'humidité comprenant :
une couche de tissu de face (14) comprenant un premier fil (23), le premier fil (23) ayant des additifs hydrofuges durables (DWR) ou une finition DWR, dans lequel le premier fil (23) comprend un polymère synthétique, le premier fil (23) formant une surface extérieure de la couche de tissu de face qui est principalement hydrophobe ;
une couche de tissu arrière (12) comprenant un deuxième fil hydrophile (18) formant un noyau de récupération d'humidité pour absorber l'humidité et la répartir sur une surface intérieure de la couche de tissu arrière (12), le deuxième fil hydrophile (18) comprenant des fibres naturelles ou des fibres cellulosiques régénérées ;
dans lequel la couche de tissu de face (14) comprend en outre un troisième fil (24) tricoté avec le premier fil (23) de telle sorte que le troisième fil (24) se trouve sur une surface intérieure de la couche de tissu de face (14) et que le premier fil (23) se trouve sur la surface extérieure de la couche de tissu de face (14), le troisième fil (24) étant un élasthanne et ayant un titre de fil compris entre 1 Tex et 8 Tex (10 D à 70 D) ;
dans lequel la couche de tissu arrière (12) comprend en outre un quatrième fil (20) tricoté avec le deuxième fil (18) de telle sorte que le quatrième fil (20) se trouve sur une surface intérieure de la couche de tissu arrière (12) et que le deuxième fil (18) se trouve sur une surface extérieure de la couche de tissu arrière (12), dans lequel le quatrième fil (20) est un élasthanne et a un titre de fil compris entre 1 Tex et 8 Tex (10 D et 70 D) ; et
un fil de liaison (16) reliant la couche de tissu avant (14) et la couche de tissu arrière (12) dans le tissu tricoté (10) de telle sorte que la surface intérieure de la couche de tissu de face (14) fait face à la surface intérieure de la couche de tissu arrière (12), le fil de liaison (16) étant un élasthanne à brin unique.

2. Tissu tricoté (10) selon la revendication 1, dans lequel le premier fil (23) est filé en utilisant les additifs DWR à l'intérieur du fil.

3. Tissu tricoté (10) selon la revendication 1, dans lequel la surface extérieure de la couche de tissu de face (14) est finie avec un revêtement DWR.

4. Tissu tricoté (10) selon la revendication 1, dans lequel le polymère synthétique est choisi parmi un groupe consistant en un nylon, un polyester, un polypropylène, un acrylique et tout mélange ou combinaison de ceux-ci.

5. Tissu tricoté (10) selon la revendication 4, dans lequel le polymère synthétique du premier fil (23) est du nylon 6.6, et le premier fil (23) a un titre de fil compris entre 2 Tex et 11 Tex (20 D - 100 D) et un nombre de filaments compris entre 10 et 186.

6. Tissu tricoté (10) selon l'une quelconque des revendications 1 à 4, dans lequel la surface extérieure de la couche de tissu de face (14) est peluchée ou brossée.

7. Tissu tricoté (10) selon l'une quelconque des revendications 1 à 6, dans lequel le quatrième fil (20) est un élasthanne de 3 Tex ou 4 Tex (30D ou 40D).

8. Tissu tricoté (10) selon l'une quelconque des revendications 1 à 7, dans lequel les fibres naturelles ou les fibres cellulosiques régénérées du deuxième fil (18) sont choisies parmi un groupe consistant en un coton, de la soie, de la laine, du modal, du micro-modal, de la viscose, du lyocell, du cupro, de la soie artificielle, des fibres cellulosiques régénérées, des fibres protéiques régénérées et toute combinaison de ceux-ci.

9. Tissu tricoté (10) selon l'une quelconque des revendications 1 à 8, dans lequel le fil de liaison (16) a un titre de fil compris entre 1 Tex et 8 Tex (10 D à 70 D).

10. Tissu tricoté (10) selon la revendication 9, dans lequel le fil de liaison (16) forme une structure en zigzag entre la couche de tissu arrière (12) et la couche de tissu de face (14).

11. Tissu tricoté (10) selon l'une quelconque des revendications 1 à 10, dans lequel le tissu est un tissu tricoté à la trame ou à la chaîne.

12. Tissu tricoté (10) selon la revendication 11, dans lequel le tissu tricoté à la trame ou à la chaîne présente une construction en simple jersey plaqué ou une construction en double jersey plaqué.

13. Tissu tricoté (10) selon l'une quelconque des revendications 1 à 12, dans lequel la surface extérieure de la couche de tissu arrière (12) comprend une finition absorbante.

14. Tissu tricoté (10) selon l'une quelconque des revendications 1 à 11 ou la revendication 13, dans lequel le tissu est un tissu piqué ou un tissu tricot.

15. Article d'habillement comprenant le tissu (10) selon l'une quelconque des revendications 1 à 14.
